

Jan. 27, 1959

S. A. HAYS

2,871,142

CHEMICAL NICKEL AND COBALT PLATING PROCESS

Filed May 20, 1955

2 Sheets-Sheet 1



FIG. 1



FIG. 2



FIG. 3

INVENTOR.  
STEPHEN A. HAYS

BY

*William L. Hays*  
ATTORNEY

Jan. 27, 1959

S. A. HAYS

2,871,142

## CHEMICAL NICKEL AND COBALT PLATING PROCESS

Filed May 20, 1955

2 Sheets-Sheet 2



FIG. 4



FIG. 5



FIG. 6



**FIG. 8**



FIG. 9



FIG. 10



FIG. II

INVENTOR.  
STEPHEN A. HAYS

BY

William R. Lane

ATTORNEY

1

2,871,142

## CHEMICAL NICKEL AND COBALT PLATING PROCESS

Stephen A. Hays, Sierra Madre, Calif., assignor to North American Aviation, Inc.

Application May 20, 1955, Serial No. 509,808

12 Claims. (Cl. 117—102)

The present invention concerns a new and novel process of chemical nickel or cobalt plating either in a batch or continuous type of operation. More particularly, the invention involves a method of maintaining the nickel or cobalt concentrations of the plating bath and of removing detrimental ions from the spent plating solution.

In U. S. Patent No. 2,532,283, Brenner and Riddell describe a batch process of chemical nickel plating in which a nickel salt (preferably nickel chloride), a hypophosphite (sodium) and a buffer salt (sodium salts of carboxylic acids or ammonium salts) make up the plating solution. The process described therein, while not expressing the optimum conditions and operating solution, forms the basis for the chemical nickel processes presently in use. Batch processes inherently present many problems when their use extends to production work. The difficulty of keeping within predetermined concentration limits and ratios, accurate pH control, and removal of various undesirable ions and by-products are all apparent in batch type operation. These above difficulties result in variations in plate quality and limit the thickness which can be continuously plated. Brenner et al., in U. S. Patent No. 2,532,284, show cobalt plating wherein cobalt chloride, sodium hypophosphite and sodium citrate are reacted with water to produce cobalt. The above difficulties are also present in cobalt plating.

In U. S. Patent No. 2,658,839, Talmey and Crehan describe a process of nickel plating using a plating bath and a reservoir, the latter containing the bulk of the plating solution. The reservoir idea provides a continuous process only by providing a much larger volume of solution, which takes longer for complete use. The reservoir concept has the advantage of storing the bulk of the solution at a lower temperature, thus preventing thermal decomposition. In contradiction to the process disclosed herein, the Talmey et al., process does not include any provision for actually regenerating the plating solution. Other prior attempts to provide a continuous system of chemical nickel or cobalt plating have all failed to prevent the gradual build-up of detrimental products in the plating solution.

The present invention involves, basically, the provision of a new and novel process which includes providing a cation exchange column in the chemical nickel or cobalt plating process. The incorporation of the improvements of the present invention prevent rapid build-up of undesirable ion concentrations and precipitates in the plating solution. The efficiency of the present invention is predicated individually and collectively on the extraction properties of cation exchange solids, on the extraction properties of the chelating or complexing anions in solution, on the counter-current extraction and on the inherent

2

close control of the complexing agent-to-nickel (or cobalt) ratio in the plating bath.

The invention as hereinafter described will be explained in terms of chemical nickel plating. The discussion thereafter is also applicable to cobalt plating. In the preferred form of the invention, the cation exchange resin is a nickel complexing agent in the solid state, which will extract nickel from an aqueous sulfate solution. The fact that the resin is a solid makes it possible to readily separate it. Flow through a column of adequate length (equivalent to multiple "batch" extractions) provides over 99.9% efficiency. For example, citrate ion is a strongly competing nickel complexing agent, such that an equilibrium distribution of nickel between the solid resin and the dissolved citrate ion would be achieved in a batch extraction. However, flow of the citrate solution through a column in the opposite direction to the flow of nickel sulfate solution used to "charge" the column with nickel, may also be used to produce over 99.9% efficiency in either of two ways: (1) in terms of citrate saturation when adequate nickel is present, or (2) in terms of complete removal of nickel when adequate citrate passes through. The preferred form of the present process utilizes the former—adequate nickel—although the nickel content and column length need be no more than sufficient to provide a nickel concentration in the emerging solution equivalent to about 95% of the citrate concentration. At the same time, the concentration of cation contaminants in the solution, such as cadmium or calcium, is continuously decreasing through the column length so that they are efficiently removed, avoiding inhibition of plating and precipitation of calcium sulfate when the solution is heated. Of course, since these are all exchange reactions, addition of nickel in this manner avoids addition of the accompanying anion (such as sulfate) and removes an equivalent amount of other cations. This provides additional savings by reducing the build-up of total solids in the solution so that it is less frequently necessary to separate the solids or discard the bath.

40 The chemical reactions and steps involved in the preferred form of the invention are as follows, where "R" represents the cation exchange resin negative radical, and underlining denotes the solid state as differentiated from the solution state:

45 (1) Charging the cation exchange column with nickel:



(2) Charging the plating solution with nickel by passing the solution through the cation exchange column:



(3) The plating reaction in which  $\text{Ni}^{\circ}$  is the plated nickel:



(4) Removing impurities of plating solution in the cation exchange column:



60 (5) Removing excess acid from plating solution:



65 The excess acid removal in (5), which exchanges hydrogen ions formed in the plating solution, occurs along

with the exchange of sodium and nickel ions in the column. Such hydrogen ion exchange varies inversely with respect to the pH and the amount of sodium ions present.

The incorporation of a cation exchanger in the electroless nickel process has many advantages. Among these is that it removes traces of bath inhibiting metal ions, such as cadmium. Further, it provides a source for introducing nickel to the bath in which both the anions, such as sulfate, and an equivalent amount of undesirable sodium ions are eliminated from the plating solution. The process also provides for an automatic control of the "nickel-to-citrate" ratio, thus avoiding frequent analysis and simplifying solution maintenance. The presence of the cation exchange column, in addition, provides a convenient apparatus for removing calcium, magnesium and other detrimental ions from the main water supply, thus permitting its substitution for the relatively expensive distilled water heretofore used in the electroless nickel process. As hereinafter explained, the column can also be used for recovering nickel from waste.

An object of this invention is to provide a new electroless nickel and cobalt plating process.

A further object of this invention is to provide a new process of chemical nickel plating.

A still further object of this invention is to provide an ion exchange column through which an electroless nickel or cobalt plating solution circulates.

An additional object of this invention is to provide a method of providing automatic control of the citrate-to-nickel ratio in a citrate-containing nickel plating bath.

A further object of this invention is to provide a continuous process of regenerating the plating solution used in electroless nickel or cobalt plating.

A still further object of this invention is to provide a process of chemically depositing nickel to form a tough, hard and adherent deposit on various metallic surfaces.

An additional object of this invention is to provide a process for the removal of calcium and cadmium inhibiting ions from an electroless nickel or cobalt plating bath.

Other objects of invention will become apparent from the following description taken in connection with the accompanying drawings, in which

Fig. 1 represents the over-all flow sheet;

And Figs. 2 to 11 illustrate the individual steps of the process in detail.

In the following example, the plating solution is assumed to contain nickel citrate and sodium hypophosphite plus water which reacts to form citric acid, sodium phosphite and nickel metal, as shown in Equation 3 above. The process of this invention serves to regenerate the nickel citrate or other nickel salt present in the plating solution. In Fig. 1, a cation exchange material, typically a resin in the form of sodium salt, is placed (as is well known in the water softening art) in an ion exchange column 50 and in two other columns 40 and 30. A tank 37 is provided to dissolve the salts used to recharge these columns. Since the columns should be kept full of water or solution, the outlets hereinafter mentioned should open between the tops of the columns and the bottom of the tank 37. In addition to the various valves shown it is to be understood that each of the columns will ordinarily have drain valves to provide for emptying the columns when required. The process comprises three major operations: first, charging the column 50 with nickel ions; second, treating the plating solution; and third, charging the columns 30 and 40 with sodium ions. Insofar as the electroless nickel plating process is concerned, the second step of treating the plating solution is the essence of the present invention. The description of the remaining flow lines, valves and auxiliary equipment shown in Fig. 1 will be explained in detail in considering the various specific steps of the process as individually illustrated in Figs. 2 to 11.

The first step in charging column 50 with nickel is to pass tap water through valve 29, flow line 31, and forward through column 30 into tank 37 to dissolve nickel sulfate in such tank. A moderately concentrated solution (200-700 grams/liter of  $\text{NiSO}_4 \cdot 6\text{H}_2\text{O}$ ) is formed in tank 37. In this operation, valves 28 and 34 are open and valve 35 is closed. Column 30 contains a cation exchange material which softens the incoming water by removing such foreign cations as calcium and magnesium therefrom. In the next charging step the nickel sulfate solution from tank 37 is passed slowly through valve 34 (valve 28 being closed), through line 44, and through column 50 in reverse. The amount of nickel added should be limited so that 95% to 100% of the nickel added will be held by column 50. The nickel sulfate solution flows through column 50, in reverse through column 40 by means of line 43, leaving any remaining nickel in column 40. When the other bath cations are sodium, the nickel ions will be exchanged for sodium ions and the effluent will emerge as a sodium sulfate solution which may be discarded to waste through line 39 and valves 13 and 36. Preferably, a transparent section is provided between columns 50 and 40 so that the nickel addition from tank 37 may be stopped when the usual green color of the nickel solution is seen passing from column 50 to column 40.

Optionally, as seen in Fig. 4, additional water may be passed forward through column 30 for softening purposes, then in reverse through columns 50 and 40 as a rinse. In Figs. 1 to 11 and the accompanying description, the term "forward" is used to denote flow in an upward direction, while "reverse" denotes flow downwardly. The present process is also capable of use if these conditions are reversed. In such a case, gas release valves will be needed above columns 40 and 50.

Fig. 5 shows in detail the main operational steps of the present process. A plating solution inlet 42 and plating solution outlet 52 are provided, the latter returning regenerated plating solution to the plating bath. It is to be understood that the process, while ordinarily of a continuous nature entailing constantly circulating the plating solution, may be of a batch type operation. The spent electroless nickel plating solution from the plating tank 60 is passed forward through column 40, line 43, and forward through column 50 and on through line 53, filter 51 and returned through outlet 52 to the plating tank 60. The filter 51 acts to retain any of the cation exchange resin which may be entrained with the regenerated plating solution. Carbon may also be employed in filter 51 to remove organics from the plating solution. The presence of a nickel complexing agent, such as sodium citrate, in the spent plating solution will result in an exchange of the nickel ions of the cation exchange material for the sodium component of the sodium citrate forming nickel citrate as in Equation 2 above. The amount of nickel removed from the exchange material is dependent upon and roughly equivalent to the amount of free or sodium citrate in the spent plating solution. When, as explained above, sufficient nickel is present in the various columns to provide for citrate saturation in terms of nickel, the ratio of equivalents of citrate-to-nickel is automatically maintained at slightly above a one-to-one ratio. This ratio is maintained until the supply of nickel in column 40 is considerably depleted. This ratio range has been found to be optimum for electroless nickel plating since high efficiency is provided with an absence of plate roughness.

Before the nickel content of a cation exchange column 50 is excessively depleted, tap water from valve 29 (Fig. 6) is passed through column 30 for softening, and then forward through columns 40 and 50 to rinse the nickel citrate out of the column. The resultant rinse solution may be used to replace evaporation losses by the immediate addition thereof to the plating solution already passed through the column or by use for addi-

tions to the treatment tanks. The rinse solution may also be used to dissolve the hypophosphite to be added to the plating solution.

Figs. 7 through 11 show a method of recharging columns 30 and 40 with sodium. These steps act to strip the ion exchange material of calcium and other foreign ions, replacing them with sodium ions. In Fig. 7, tap water from valve 29 is softened by passing it through line 31 and column 30 into tank 37 to prepare, typically, a saturated solution of sodium chloride. This step is the same as the step illustrated in Fig. 2, except for substitution of a sodium salt for the nickel salt. The same tank 37 may be used for this operation, although it is generally more convenient to have separate tanks available for storing both the sodium and nickel salt solutions.

Fig. 8 illustrates the step of passing the concentrated sodium salt solution slowly in reverse through column 30 and out to waste through a sewage outlet 33.

Fig. 9 shows column 30 being rinsed forwardly with tap water from valve 29, which rinse water is disposed in sewage outlet valve 36. Rinsing is done forwardly in Fig. 9. An excess of sodium salt solution is used in Fig. 8 in order to simplify the apparatus and avoid leaving foreign cations from the tap water at the wrong end of column 30. The next step in charging columns 30 and 40 is to pass the concentrated sodium salt solution slowly in reverse through column 40 and lines 44, 41 and 39 to the sewage outlet valve 36. As seen in Fig. 11, tap water is then passed forward through column 30 for softening purposes, then in reverse through column 40 to rinse the sodium salt solution and the displaced cations from the column and to discard the effluent to waste through line 39 and sewage outlet valve 36.

When all of the nickel which is plated from the solution is to be replaced by regeneration in column 50, the frequency of recharging the column with nickel can be estimated from the column capacity and the amount of plating. The hardness of the available water supply determines the frequency of recharging column 30. The calcium, cadmium and other cations (other than sodium) are deposited from the plating solution almost entirely in column 40. These are then carried to waste when displaced by concentrated sodium sulfate left from exchange of concentrated nickel sulfate addition solution during recharging with nickel. However, a nickel concentration sufficient to completely remove these other cations would also result in excessive loss of nickel. Therefore, when more complete removal of the foreign cations is desired, a concentrated solution of a sodium salt is passed through column 40 (in reverse) to waste, after the solution containing free citrate has been passed forward through the same column to selectively remove the nickel. The routine treatment of used plating solution, as in Fig. 5, fulfills the latter requirement and completely avoids loss of nickel.

As seen in Fig. 8, a concentrated sodium salt solution is passed through column 30, in reverse, to recharge it and to replace calcium and other detrimental cations with sodium. Complexing agents, such as ethylene diamine tetracetate, may also be passed in reverse through one or more of the columns 39, 40 or 50 to remove any additional foreign cations. Such agents may be passed through column 50 so long as they do not waste excessive amounts of nickel.

As in the past used processes of chemical nickel or cobalt plating, the present process may be used to plate workpieces of a metal or alloys thereof selected from the group consisting of iron, platinum, silver, gold, cobalt, palladium, nickel, aluminum, copper and titanium. In general, each of these metals must be cleaned by conventional procedures before the electroless nickel or cobalt plating treatment. The pretreatment of these various metals and their alloys is fully set out in the Brenner and Riddell patents, supra. Electroless nickel and cobalt may also be plated directly on graphite or on glass or plastics

if such materials are made conductive or precoated with a catalytic metal such as iron or aluminum.

Various types of commercially available cation exchange mediums may be used for filling columns 30, 40 and 50. Generally, among these, the nuclear sulphonate type, the phenolic methylene sulphonate type, carboxylic and aluminum silicate type mediums may be used. Specifically, Amberlite IR-120, produced by Rohm and Haas Company, and Dowex-50, manufactured by the Dow Chemical Company, are examples of cation exchange resins suitable for the use in the present process.

The preferred bath composition and characteristics are set out below in Table I.

Table I

| 15 | Bath composition           | Range       | Preferred  |
|----|----------------------------|-------------|------------|
| 20 | Ni <sub>3</sub> citrate    | 0.05N-2.0N  | 0.20-0.5N. |
|    | Na hypophosphite           | 0.15N-0.30N | 0.23N.     |
|    | pH                         | 3.0-5.0     | 3.9-4.1.   |
|    | Ratio of citrate to nickel | 1.0-2.0     | 1.1-1.2.   |
|    | Deposition rate, mil/hr    | 0.1-1.0     | 0.5.       |
|    | Bath temperature           | 180°-212° F | 210° F.    |
|    | Plating time               | As required |            |
|    | Column temperatures        | 50-170° F   | 50-140° F. |

25 The present invention is not limited to the nickel, cobalt and sodium salts heretofore specifically mentioned. The salts may also be the chlorides, nitrates, carbonates, or any other soluble salts which are not tightly complexed. The anions associated with the various salts are washed through the various columns during operation of the process. Whereas the complexing agent for the nickel has been herein described and explained in terms of the citrate, such compounds as the hydroxyacetates, gluconates, succinates, or malonates may also be used. These agents may be termed hydroxy carboxylates. Furthermore, amino compounds such as triethylamine or ethanolamine may be employed as the complexing agent. Potassium salts may be substituted for the sodium salts used in the regeneration process.

30 When it is desired to adapt the disclosed process to cobalt plating baths, the pH of the solution will normally be from 8-10 as prescribed by Brenner and Riddell, supra. An excess of sodium citrate or other complexing agent mentioned above, or the sodium potassium tartrate discussed in Brenner et al., should be used to insure holding and complexing the cobalt salt in solution. Furthermore, to prevent precipitation in the ion exchange column of hydroxides, which are added to keep the cobalt plating bath at the desired pH, the circulating cobalt

35 plating solution may be acidified before its entrance into the column and the pH readjusted to alkaline as the regenerated solution is recirculated to the plating bath. The parts by weight of cobalt ion, hypophosphite radical complexing radical, and water may be in the ranges expressed in the Brenner et al., patent.

40 In Fig. 1, column 50 is the only essential column. Column 30 is used mainly for water softening purposes and can be recharged in the standard manner for such columns. Such column can be entirely eliminated if a tank or other source of soft water is available to dissolve the nickel or cobalt salt and rinse the other columns in the reverse direction. Soft water may be obtained by passing ordinary water forward through column 40 and/or column 50 after they have been thoroughly rinsed. Column

45 40 is essentially an extension of column 50 separated to simplify visual control of the amount of nickel added and to permit displacement of foreign cations to waste by sodium ions only in that end of the column where the nickel or cobalt is minimized and most of the foreign cations are concentrated. The hypophosphite, citrate radical and phosphite are essentially unaffected by their passage through the cation exchange column or columns.

50 Although the invention has been described and illustrated in detail, it is to be clearly understood that the same is by way of illustration and example only and is

not to be taken by way of limitation, the spirit and scope of this invention being limited only by the terms of the appended claims.

I claim:

1. A process of treating an electroless nickel process plating solution containing nickel citrate and sodium hypophosphite in which the plating process depletes the nickel ions in said nickel citrate and forms sodium citrate and hydrogen ions in said solution, said treating process comprising passing the depleted plating solution continually through a nickel-charged cation exchange medium, exchanging the nickel ions in said medium with the sodium ions and hydrogen ions in the depleted plating solution, and recirculating the resultant nickel citrate solution to said electroless nickel plating process and maintaining the ratio of equivalents of citrate-to-nickel at 1.0 to 2.0.

2. The process as set out in claim 1 in which the nickel salt of a complexing agent is nickel citrate, the hypophosphite is sodium hypophosphite and the ratio of equivalents of nickel-to-citrate in the circulating solution is maintained at approximately 1:1.

3. A method of regenerating an electroless nickel plating process bath containing an aqueous solution of a nickel salt of a nickel complexing agent selected from the class consisting of carboxylate and amino compounds, an alkali metal hypophosphite and impurities including calcium and cadmium ions, an alkali metal salt of the nickel complexing agent and hydrogen ions being formed in the plating process, comprising circulating said solution through a nickel-charged cation exchange material, exchanging nickel ions from said material with the alkali metal ions of the complexing agent and the hydrogen ions, extracting calcium, cadmium ions from said solution and recirculating said solution to said plating process bath, and maintaining the ratio of equivalents of said complexing agent-to-said nickel in the range of from 1.0 to 2.0.

4. The process of electroless plating a metal selected from the class consisting of cobalt and nickel on a metal-surface workpiece comprising providing an aqueous solution of metal ions of said class and a complexing agent selected from the class consisting of carboxylates and amino compounds in amounts such that the ratio of equivalents of said complexing agent-to-said metal is in the range of from 1.0 to 2.0, and an alkali metal hypophosphite, immersing the workpiece in said solution for a time sufficient to give a desired plating thickness on said workpiece, circulating said solution through a cation exchange medium containing cations of a metal of said class, and contacting said medium with said solution whereby said solution is recharged with the metal cations from said medium and maintaining said complexing agent-to-said metal ratio.

5. The process of chemical nickel plating a metal-surfaced workpiece comprising providing an aqueous solution of nickel ions and a carboxylate complexing agent having from 2 to about 6 carbon atoms in amounts such that the ratio of equivalents of said complexing agent-to-nickel is in the range of from 1.0 to 2.0, and an alkali metal hypophosphite, immersing the workpiece in said solution for a time sufficient to give a desired plating thickness of nickel metal on said workpiece, circulating said solution through a nickel-charged cation exchange medium, and contacting said medium with said solution whereby said nickel solution is recharged with nickel ions from said medium and maintaining said complexing agent-to-said metal ratio.

6. The process of claim 5 in which the complexing agent is a citrate and the hypophosphite is sodium hypophosphite.

7. The process of claim 5 in which the complexing agent is a citrate, the hypophosphite is sodium hypophosphite, and the ratio of equivalents of complexing agent-to-nickel is substantially 1:1.

8. The process of chemical nickel plating a metal-surfaced workpiece comprising providing an aqueous solution of nickel ions and a complexing agent selected from the class consisting of carboxylates and amino compounds in amounts such that the ratio of equivalents of said complexing agent-to-said metal is in the range of from 1.0 to 2.0, and an alkali metal hypophosphite, immersing the workpiece in said solution for a time sufficient to give the desired plating thickness of nickel metal on said object, and intermittently circulating said solution through a nickel-charged cation exchange medium and contacting said medium with said solution whereby said solution is regenerated with nickel ions from said medium and maintaining said complexing agent-to-said metal ratio.

9. The process of chemical nickel plating a metal-surfaced workpiece comprising providing an aqueous solution of nickel ions and a complexing agent selected from the class consisting of carboxylates and amino compounds in amounts such that the ratio of equivalents of said complexing agent-to-nickel is in the range of from 1.0 to 2.0, and an alkali metal hypophosphite, immersing the workpiece in said solution for a time sufficient to give the desired plating thickness of nickel metal on said object, and continuously circulating said solution through a nickel-charged cation exchange medium and contacting said medium with said solution whereby said solution is regenerated with nickel ions from said medium, intermittently passing a sodium salt solution through said medium to remove foreign ions therefrom and intermittently recharging said medium with nickel ions by passing a nickel sulfate solution therethrough and maintaining said complexing agent-to-said metal ratio.

10. A process of chemical nickel plating an object of a metal chosen from the group consisting of iron, platinum, silver, gold, cobalt, palladium, aluminum, titanium, copper and nickel, comprising the steps of exposing said object to an aqueous solution of nickel ions and a carboxylate complexing agent having from 2 to about 6 carbon atoms in amounts such that the ratio of equivalents of said complexing agent-to-said metal is in the range of from 1.0 to 2.0, and an alkali metal hypophosphite for a time sufficient to give a predetermined plating thickness of nickel metal, continually circulating the aqueous solution through a nickel complexing cation exchange medium, saturating the nickel complexing agent solution with nickel cations, intermittently flowing a sodium salt solution through said cation exchange medium to remove foreign cations from the exchange medium, and intermittently counter-current flowing a nickel sulfate solution through said cation exchange medium to recharge said medium with nickel cations.

11. A method of regenerating an electroless nickel and cobalt plating bath containing an aqueous solution of metal ions selected from the class of cobalt and nickel, a complexing agent selected from the class consisting of carboxylates and amino compounds, and an alkali metal hypophosphite, comprising circulating said aqueous solution through a cation exchange column charged with metal ions of said class to replace the metal ions expended in the plating process and maintaining the ratio of equivalents of said complexing agent-to-said metal ions in the range of from 1.0 to 2.0.

12. A process of treating an electroless nickel and cobalt process plating solution containing metal ions selected from the class consisting of cobalt and nickel, a complexing agent selected from the class consisting of carboxylates and amino compounds, and an alkali metal hypophosphite, in which the plating process depletes the nickel and cobalt cations in said solution, forms hydrogen ions, and leaves alkali metal cation salts in said solution, said treating process comprising passing the depleted plating solution through a cation exchange medium charged with metal ions of said class, exchanging the metal ions in said medium with the alkali metal ions and hydrogen ions in the depleted solution, recirculating the resultant

solution to said electroless nickel plating process, and maintaining the ratio of equivalents of said complexing agent-to-said metal ions in the range of from 1.0 to 2.0.

References Cited in the file of this patent

UNITED STATES PATENTS

2,532,283 Brenner et al. Dec. 5, 1950  
2,726,968 Spaulding Dec. 13, 1955

OTHER REFERENCES

Costa: Industrial and Engineering Chemistry, vol. 42, No. 2, February 1950, pp. 308-311.

Kunin et al.: Ion Exchange Resins (1950), John Wiley & Son, Inc., N. Y., pp. 135, 139.

Paulson et al.: Plating, vol. 40, No. 9, September 1953, pp. 1005-1009.